

March 19, 1968

HAKARU MASUMOTO ET AL 3,374,123  
METHOD OF MANUFACTURING NONMAGNETIC, ELASTIC ARTICLES  
HAVING A SMALL CHANGE OF VIBRATION AND  
DEFLECTION FOR TEMPERATURE CHANGE

Filed March 3, 1965

3 Sheets-Sheet 1

Fig. 1.



INVENTORS

HAKARU MASUMOTO  
TAKEO KOBAYASHI  
*Irvin S. Thompson*

BY

ATTORNEY

March 19, 1968

HAKARU MASUMOTO ET AL 3,374,123  
METHOD OF MANUFACTURING NONMAGNETIC, ELASTIC ARTICLES  
HAVING A SMALL CHANGE OF VIBRATION AND  
DEFLECTION FOR TEMPERATURE CHANGE

Filed March 3, 1965

3 Sheets-Sheet 2

Fig. 2



INVENTORS

HAKARU MASUMOTO  
TAKEO KOBAYASHI

BY

*Ivan S. Thompson*

ATTORNEY

March 19, 1968

HAKARU MASUMOTO ET AL. 3,374,123  
METHOD OF MANUFACTURING NONMAGNETIC, ELASTIC ARTICLES  
HAVING A SMALL CHANGE OF VIBRATION AND  
DEFLECTION FOR TEMPERATURE CHANGE

Filed March 3, 1965

3 Sheets-Sheet 3

Fig. 3.



INVENTORS

HAKARU MASUMOTO  
TAKEO KOBAYASHI

BY *Irvin S. Thompson*

ATTORNEY

1

3,374,123

**METHOD OF MANUFACTURING NON-MAGNETIC, ELASTIC ARTICLES HAVING A SMALL CHANGE OF VIBRATION AND DEFLECTION FOR TEMPERATURE CHANGE**

Hakaru Masumoto, Sendai, and Takeo Kobayashi, Natori, Japan, assignors to The Foundation, The Research Institute of Electric and Magnetic Alloys, Sendai, Japan  
Filed Mar. 3, 1965, Ser. No. 436,902  
Claims priority, application Japan, Mar. 4, 1964,

39/11,779

3 Claims. (Cl. 148—11.5)

**ABSTRACT OF THE DISCLOSURE**

A method of manufacturing non-magnetic and elastic articles having little change in Young's modulus with change in temperature, which comprises annealing an alloy consisting essentially of about 50% gold and about 50% palladium by heating said alloy at a temperature above 600° C. for at least one minute, and then heat treating said alloy by a suitable combination of quenching, cold working, and tempering.

This invention relates to a process for the manufacture of non-magnetic and elastic body consisting essentially of about 50% by weight of palladium and about 50% by weight of gold.

The principal object of the invention is to provide a non-magnetic and elastic body having an arbitrary value of the temperature coefficient of Young's modulus (or rigidity modulus), between from an ordinary negative value, say  $-20 \times 10^{-5}$ , to a certain positive value, say about  $+5 \times 10^{-5}$ , a high resistance against oxidation and corrosion, and a hardness of various degrees.

In conventional methods of manufacturing elastic articles having a small temperature change of vibration and deflection, elinvar type alloys (Fe-Ni alloys added with other elements) and co-elinvar type alloys (Fe-Co alloys added with other elements) have been used.

All the above known alloys, however, show not only ferromagnetic properties but also have disadvantage of causing corosions when exposed to an acidic or alkaline vapour or solution or to a solution of salts. Accordingly, hitherto conventional alloys are not suitable for certain applications.

As a result of a number of investigations and experiments to obviate the above disadvantage of conventional alloys, the inventors discovered that palladium-gold alloys have not only high resistances against oxidation and corrosion but also non-magnetic properties as well as a hardness of various degrees. Alloys of the invention obviate the disadvantage inherent to conventional elastic alloys.

A process of manufacturing the elastic articles according to the invention is characterized in that a binary alloy consisting essentially of about 50% by weight of palladium and about 50% by weight of gold is subjected to one of the following several kinds of treatment:

(1) An alloy annealed at a temperature above 600° C. is quenched by rapidly cooling it at a rate faster than 1° C./second and then heated at a comparatively low temperature, such as 200 to 550° C.;

(2) An alloy annealed at a temperature above 600° C. is cold worked to reduce the sectional area more than 20% at room temperature and then heated at a comparatively low temperature, such as 200 to 550° C.;

(3) An alloy annealed at a temperature above 600° C. is first quenched by rapidly cooling it at a rate faster than 1° C./second and then cold worked to reduce the sectional area more than 20% at room temperature and

2

lastly heated at a comparatively low temperature, such as 200 to 550° C. The article thus obtained has an arbitrary value of temperature coefficient of Young's modulus (or rigidity modulus) ranging from an ordinary negative value to a positive value and different values of hardness.

The principles of the invention will now be explained further in detail. According to the invention, at first, a mixture consisting of a proper amount of palladium and gold or in addition suitable amount of said sub-ingredients is melted in air, in vacuo, or in an inert gas by means of a suitable furnace, then degassed by adding a small quantity of degassing agent (element) such as manganese, silicon aluminum, titanium, etc., and stirred thoroughly to produce a melted alloy having homogeneous structure. Then the melted alloy is poured into a mould of suitable size and shape to obtain a sound ingot, and the ingot thus prepared can be forged, rolled, swaged or drawn at room temperature or at an elevated temperature lower than 1400° C. to provide a product having desired shape and size.

Thereafter, the product is heated for more than 1 minute, say 1 hour, at a temperature higher than 600° C. but lower than the melting point of the alloy and then gradually cooled. If desired, the mechanical strength of the product can be increased by several means for instance by quenching from a temperature higher than 400° C. but lower than the melting point of the alloy or by cold working at a reduction ratio more than about 20% or by applying both quenching and cold working. If further stabilization of characteristics is desired, the product can be heated at a temperature higher than 200° C. but lower than 550° C. for at least one minute after the above quenching or cold working or application of both quenching and cold working. The final product thus obtained shows an arbitrary value of temperature coefficient of Young's modulus (or rigidity modulus) ranging from an ordinary negative value to a positive value.

For a better understanding of the invention reference is made to the accompanying drawings, in which

FIG. 1 is a diagram illustrating densities (at 20° C.), Young's moduli (at 20° C.), mean temperature coefficients (0-40° C.) of Young's modulus (0-40° C.) and mean thermal expansion coefficients (0-40° C.) of palladium-gold alloys for different concentration of palladium in said alloys;

FIG. 2 is a diagram illustrating mean temperature coefficients of Young's modulus (0-40° C.) of three kinds of alloys which were processed through cold swaging at a reduction ratio of 96%, for different annealing temperatures; and

FIG. 3 is a diagram illustrating relations between natural frequencies and temperature of three kinds of alloys which were annealed at 360° C. for 15 hours after cold swaged for 96% reduction.

The invention will now be further explained in detail by examples. A mixture of palladium and gold was at first melted in an alumina crucible of about 10 mm. inside dia. by means of a Tammann furnace (electric resistance furnace) while passing hydrogen gas, then the mixture was stirred thoroughly and cooled in said crucible. Then the ingot was made into a bar of about 2 mm. dia. by swaging at a reduction ratio of 96% at room temperature, and a portion of the bar, about 10 cm. long, was cut off to provide a sample to determine behaviours in the state of cold working. The sample was then heated at various temperatures for 15 hours and cooled to take measurements. At last, the sample was annealed at 1000° C. for one hour and then measurements were made. Young's moduli were determined by measuring at first natural frequencies of the sample bars by means of a device, based on principles of an electrostatic vibrator controlled oscillator, and then by calculation from the

measured values. Thermal expansion coefficients of the sample bars in the neighbourhood of room temperature were determined by means of a precise vertical dilatometer. Mean temperature coefficients of Young's modulus (0-40° C.) for different compositions of alloys were calculated based on the above measured values and densities, and the results are shown as curves in FIG. 1. The curve *a* in FIG. 1 indicates the values of mean temperature coefficients of Young's modulus at annealed conditions, that is to say the conditions when the sample bars being gradually cooled at a rate of 300° C. per hour after heated at 1000° C. for one hour. The curve *b* indicates the values for conditions after processed through cold swaging at a reduction ratio of 96%, and the curve *c* for conditions after heating the sample bars of the curve *b* at 360° C. for 15 hours.

FIG. 2 illustrates how the mean temperature coefficients of Young's modulus in the range of 0 to 40° C. vary for the different annealing temperatures. FIG. 3 illustrates how natural frequencies of three kinds of Pd-Au alloys annealed at 360° C. for 15 hours following cold working vary for different measuring temperatures.

As shown in FIG. 1, the temperature coefficients of Young's modulus of annealed alloys consisting essentially of 30 to 70% of palladium and 70 to 30% of gold lie within a range of from  $-18.0 \times 10^{-5}$  to  $-3.0 \times 10^{-5}$  when the temperature of the alloy is in the neighbourhood of room temperature, especially said coefficient of the alloys consisting essentially of 57 to 37% of palladium and 43 to 63% of gold is substantially small.

As shown in FIG. 1, the temperature coefficients of Young's modulus of alloys of the invention after processed through cold working are larger in negative domain than those of said alloys under annealed conditions, however, when said cold worked samples are annealed once again at a temperature approximately 360° C. for 15 hours the negative values of said coefficients are substantially reduced, especially said coefficient of the alloy consisting essentially of 50% of palladium and 50% of gold becomes  $+2.8 \times 10^{-5}$ . Besides, after the additional annealing following cold working, the natural frequencies of the alloys of the present invention vary in a substantially linear relationship with temperatures as shown in FIG. 3 as long as the temperature lies in the neighbourhood of room temperature, which is also a salient feature of the alloys of the invention compared with conventional elinvar type alloys showing a considerable non-linear variation of characteristic frequencies when temperature varies in the neighbourhood of room temperature (see FIG. 3).

The alloys of the invention are also characterized in having non-magnetic properties. Non-magnetic materials having constant values of Young's modulus for the temperature change have never been invented heretofore, and the alloys of the present invention are the first of the kind. In addition, the alloys of the invention have substantially strong resistances against oxidation and corrosion.

Effects of the sub-ingredients on the properties of palladium-gold alloys are shown in Table 1. It is apparent from Table 1 that additions of other elements into palladium-gold alloys generally result in a substantial increase in hardness both under the annealed condition and under the condition when heated at 360° C. following cold swaging, irrespective of the fact that the temperature coefficients of Young's modulus are caused to increase in the negative domain by said additions. The increase in hardness means the increase in yield point, which is very preferable for application of the alloys to springs.

It can be emphasized here that application of quenching from an elevated temperature or a combination of quenching and cold working to the alloys of the invention results in similar effects as those due to said cold working.

TABLE 1

| Alloys, 50%                                | As annealed<br>at 1,000° C.<br>for 1 hour          |                                                                                           | As heated at 360° C.<br>for 15 hrs. after<br>96% cold-reduction              |                                                                   |
|--------------------------------------------|----------------------------------------------------|-------------------------------------------------------------------------------------------|------------------------------------------------------------------------------|-------------------------------------------------------------------|
|                                            | Temperature<br>of Young's<br>modulus<br>(0-40° C.) | Micro-<br>coefficient<br>of Vicker's<br>hardness<br>(20° C.), 89<br>$-3.0 \times 10^{-5}$ | Temperature<br>of Young's<br>modulus<br>(0-40° C.),<br>$+2.8 \times 10^{-5}$ | Micro-<br>coefficient<br>of Vicker's<br>hardness<br>(20° C.), 184 |
| 5 Pd-50% Au alloy                          |                                                    |                                                                                           |                                                                              |                                                                   |
| 10 Aforesaid alloy<br>with addition<br>of— |                                                    |                                                                                           |                                                                              |                                                                   |
| 3.0% Pt.....                               | -9.8                                               | 116                                                                                       | -7.5                                                                         | 212                                                               |
| 1.0% Ir.....                               | -11.0                                              | 138                                                                                       | -4.7                                                                         | 249                                                               |
| 3.0% In.....                               | -11.5                                              | 100                                                                                       | -9.9                                                                         | 245                                                               |
| 3.0% Ta.....                               | -13.1                                              | 128                                                                                       | -9.3                                                                         | 258                                                               |
| 3.0% Ag.....                               | -10.5                                              | 100                                                                                       | -9.5                                                                         | 210                                                               |
| 3.0% Fe.....                               | -15.0                                              | 126                                                                                       | -10.2                                                                        | 278                                                               |
| 3.0% Ni.....                               | -14.0                                              | 144                                                                                       | -6.7                                                                         | 268                                                               |
| 3.0% Co.....                               | -11.1                                              | 123                                                                                       | -9.9                                                                         | 273                                                               |
| 1.0% Cr.....                               | -13.5                                              | 101                                                                                       | -11.2                                                                        | 260                                                               |
| 3.0% Mn.....                               | -10.0                                              | 112                                                                                       | -8.0                                                                         | 212                                                               |
| 3.0% Cu.....                               | -11.0                                              | 93                                                                                        | -7.3                                                                         | 241                                                               |
| 1.0% V.....                                | -10.0                                              | 118                                                                                       | -7.3                                                                         | 269                                                               |
| 3.0% Mo.....                               | -13.0                                              | 143                                                                                       | -8.5                                                                         | 291                                                               |
| 3.0% W.....                                | -14.0                                              | 134                                                                                       | -11.0                                                                        | 263                                                               |
| 0.2% Al.....                               | -14.0                                              | 127                                                                                       | -9.8                                                                         | 277                                                               |
| 3.0% Sb.....                               | -8.0                                               | 124                                                                                       | -5.5                                                                         | 289                                                               |
| 3.0% Sn.....                               | -13.0                                              | 107                                                                                       | -5.6                                                                         | 261                                                               |
| 3.0% Zn.....                               | -13.5                                              | 109                                                                                       | -6.5                                                                         | 242                                                               |
| 0.2% Ti.....                               | -11.0                                              | 122                                                                                       | -6.0                                                                         | 248                                                               |
| 0.1% Si.....                               | -10.0                                              | 132                                                                                       | -6.7                                                                         | 267                                                               |
| 1.0% Cd.....                               | -9.0                                               | 140                                                                                       | -7.4                                                                         | 233                                                               |
| 0.5% Be.....                               | -14.7                                              | 128                                                                                       | -11.1                                                                        | 267                                                               |
| 0.5% Zr.....                               | -11.0                                              | 117                                                                                       | -6.0                                                                         | 250                                                               |
| 0.1% B.....                                | -15.5                                              | 112                                                                                       | -11.0                                                                        | 216                                                               |
| 1.0% Nb.....                               | -15.0                                              | 105                                                                                       | -5.4                                                                         | 216                                                               |

As shown in the foregoing descriptions, temperature coefficients of Young's modulus of the alloys of the invention are not only small but also practically constant at different temperatures in the neighbourhood of room temperature. Furthermore, the alloys of the invention have nonmagnetic properties and substantially high resistances against oxidation and corrosion. Therefore, the alloys of the invention are most suitable to devices which require constant frequencies regardless of ambient temperature variation and non-magnetic properties, such as hair 35 springs of chronometers, standard tuning forks, etc.

In order to obtain a sound ingot, better forgeability and better mechanical properties of materials according to the invention, the alloys consisting essentially of palladium and gold can be added with 0 to 3% of one or more elements selected from the group consisting of platinum, iridium, indium, tantalum, silver, iron, nickel, cobalt, chromium, manganese, copper, vanadium, molybdenum, tungsten, aluminium, antimony, tin and zinc and 0 to 2% of more than one elements selected from the group consisting of titanium, silicon, cadmium, beryllium, zirconium, boron and niobium as sub-ingredients.

What we claim is:

1. A method of manufacturing nonmagnetic and elastic articles having little variation in Young's modulus 55 upon temperature change, comprising the steps of annealing a gold-palladium alloy consisting essentially of about 50% by weight of gold and about 50% by weight of palladium by heating it at a temperature higher than 400° C. but lower than the melting point of the alloy for more than one minute, quenching by cooling it at a rate faster than 1° C. per second, and tempering by further heating it at a temperature between 200° C. and 550° C. for at least one minute.
2. A method as claimed in claim 1, and between said annealing and tempering steps working said alloy at room temperature to reduce its cross-sectional area by more than about 20%.
3. A method of manufacturing nonmagnetic and elastic articles having little variation in Young's modulus upon 70 temperature change, comprising the steps of annealing a gold-palladium alloy consisting essentially of about 50% by weight of gold and about 50% by weight of palladium by heating it at a temperature higher than 400° C. but lower than the melting point of the alloy for more than one minute, then working it at room temperature to re-

duce its cross-sectional area by more than about 20%, and tempering by further heating it at a temperature between 200° C. and 550° C. for at least one minute.

**References Cited****UNITED STATES PATENTS**

2,780,543 2/1957 Schneider et al. 75-172

**OTHER REFERENCES**

The Platinum Metals and Their Alloys, Vines, 1941, pp. 34-42, 110-112.

5 DAVID L. RECK, *Primary Examiner.*

H. F. SAITO, *Assistant Examiner.*